

Patented May 5, 1925.

1,536,725

## UNITED STATES PATENT OFFICE.

PAUL ONNERTZ, OF BERLIN-WILMERSDORF, GERMANY, ASSIGNOR TO ACTIEN GESELLSCHAFT FÜR ANILIN FABRIKATION, OF BERLIN, GERMANY.

### PROCESS FOR DYEING FURS, SKINS, HAIRS, FEATHERS, OR THE LIKE.

No Drawing. Application filed November 22, 1924. Serial No. 751,676.

To all whom it may concern:

Be it known that I, PAUL ONNERTZ, a citizen of the German Republic, residing at Berlin-Wilmersdorf, Germany, have invented certain new and useful Improvements in Processes for Dyeing Furs, Skins, Hairs, Feathers, or the like, of which the following is a specification.

Furs, feathers or the like have been dyed with aid of 1.2-diaminobenzene or with 2-chloro-1.4-diaminobenzene. By the present invention tints which differ considerably from those obtained with the aforesaid compounds may be obtained by applying to the furs, skins, hairs, feathers or the like 4-chloro-1.2-diaminobenzene in presence of an oxidizing agent; the olive-brown shades thus obtained are of an excellent fastness. The skins may be mordanted or not before dyeing.

The following example illustrates the invention:

The well-washed skin is handled for some hours in a mordanting bath containing per litre

2 grams of potassium bichromate  
0.25 gram of crystallized copper sulfate  
2 grams of acetic acid of 30 per cent strength

30 or

4 grams of crystallized copper sulfate  
2 grams of acetic acid of 30 per cent strength

or  
4 grams of crystallized ferrous sulfate 35  
2 grams of acetic acid of 30 per cent strength.

The mordanted skin is handled for 4 hours in a bath containing per litre 2 grams of 4-chloro-1.2-diaminobenzene and 20 grams of 40 hydrogen peroxide solution (of about 3 per cent strength), at ordinary temperature. The skin is then well washed and finished as usual.

Having now particularly described and 45 ascertained the nature of my invention and in what manner the same is to be performed, I declare that what I claim is,

A process for dyeing furs, skins, hairs, feathers or the like consisting in treating 50 the material to be dyed with a solution of 4-chloro-1.2-diaminobenzene in the presence of an oxidizing agent.

In testimony whereof I affix my signature in presence of two witnesses.

PAUL ONNERTZ.

Witnesses:

WLAD ENDERY,  
ROY J. FOX.